

Dec. 25, 1951

N. CORSINI

2,579,551

ELECTROLYTIC PROCESS AND APPARATUS FOR MAKING COPPER DUST

Filed July 28, 1947

Fig. 1.



Fig. 2.



Fig. 3.



INVENTOR,

*Neri Corsini*

*Glascraft Downing Ltd*

ATTORNEYS

## UNITED STATES PATENT OFFICE

2,579,551

ELECTROLYTIC PROCESS AND APPARATUS  
FOR MAKING COPPER DUST

Neri Corsini, Firenze, Italy

Application July 28, 1947, Serial No. 764,213  
In Italy June 8, 1945Section 1, Public Law 690, August 8, 1946  
Patent expires June 8, 1965

3 Claims. (Cl. 204—108)

## 1

This invention relates to an electrolytic process and apparatus for making copper dust or powder.

More particularly the invention relates to a method and apparatus for producing copper dust that is especially suitable for the making of copper sulphate.

It is a primary object of this invention, therefore, to provide a process of electrolytically producing readily oxidizable copper dust or powder.

Specifically the invention has for an object to provide an electrolytic process of producing copper dust in which the rate of anodic dissolution is regulated to be substantially equal to the rate of cathodic deposition.

A still more specific object is to provide an electrolytic process of producing copper dust including the step of interposing a perforated lead plate anode between a copper anode and a cathode to maintain the concentration of cupric ions in an electrolyte substantially constant throughout the electrolysis.

A further object is to provide an electrolytic cell for carrying out the above process.

In known processes of producing copper sulphate copper grains are treated with sulphuric acid in the presence of oxidizers, such as air admixed with steam. In electrolytic methods heretofore proposed and practiced an alkaline sulphate has been employed as an electrolyte. The copper treated anodically is precipitated in the cathode space as a hydrate which is transformed into carbonate and then into sulphate by treatment with sulphuric acid. In such arrangements the cathode space must be protected with diaphragms.

However, with my invention applied to the production of copper sulphate a simplified industrial process of preparing the same comprises, cathodically depositing copper in the form of a very fine, readily oxidizable dust as set forth herein-after, oxidizing the dust at about 500° C. to about 600° C. and dissolving the copper oxide so formed in sulphuric acid.

The method and apparatus for electrolytically producing the readily oxidizable copper dust or powder will be more particularly described as follows:

Employing a cathodic current density range of about 600 to about 800 amps. per sq. m., and electrolyzing an electrolyte containing free sulphuric acid and Cu<sup>++</sup> at a low concentration, a very fine metallic dust is deposited on the cathode and precipitates to the bottom of the electrolytic cell utilized. To render this process con-

## 2

tinuous it is necessary that the anode constitute metallic copper, in practice copper scrap is utilized, which copper anode attacked by the acid dissolves to form Cu<sup>++</sup> ions.

There is, however, one difficulty, in that the yield of anodic current is practically quantitative while the cathodic is notably lower. There is therefore a continuous increase in the quantity of copper dissolved in the electrolyte so that when 10 a certain limit is reached which limit is dependent on all the conditions of electrolysis, the copper is no longer deposited at the cathode in the form of a fine dust, but as a compact deposit. To overcome this disadvantage, a cell is employed 15 in which the soluble copper anode, in practice copper scraps, is largely screened from the cathode by a lead plate having a certain number of perforations provided therein. This lead plate functions as an insoluble anode and has the 20 effect of decreasing the rate of anodic dissolution of the copper until the rate of dissolution substantially equals the rate of cathodic deposition of the copper dust. Thus a practically unvaried concentration of Cu<sup>++</sup> is maintained in the electrolyte.

The exact regulation is obtained by increasing or reducing in any suitable manner the number and size of the perforations in the lead anode. For instance, the holes in the upper part of the 30 lead plate may be made larger than those in the lower part and the level of the electrolyte in the cell raised or lowered so as to cover or to uncover them.

One construction of a cell embodying a single cathode which embodies the above described features is illustrated in the attached drawing, in which:

Figure 1 is transverse section of the cell,  
Figure 2 a longitudinal section thereof, and  
Figure 3 a diagrammatic perspective view of the same.

The cell is formed from wood or iron or other suitable material, and is lined inside with material which is not liable to corrosion by acid and 45 is a good conductor of current, for example, lead. The cathode 1 is constituted by a plate of aluminum or of copper. The anode space or compartment 2, where the metallic copper anode will be placed, is confined at the sides by the walls of the cell, whilst in front of the cathode 1 the anode space is screened by a lead plate 3, constituting the insoluble anode, in which are formed holes or perforations 4 which provide free passages 50 between the anode space 2 and the cathode 1. 55 These holes are more numerous and larger on the

upper part of the plate. Therefore, by raising or lowering the level of the electrolyte a little so as to cover more or less the larger holes the concentration of  $Cu^{++}$  in the electrolyte can be increased or diminished at will thus keeping the concentration within the desired limits. The metallic dust which separates gathers in the well or bottom 5 of the cell and is extracted by suitable means. All the cell is under a positively charged tension. Therefore, the copper dust which is deposited on the bottom is also positively charged, however, the amount that is redissolved is negligible.

The walls of the cell can be lined internally with material that is not subject to corrosion by acid and is non-conductive, such as ebonite, rubber, synthetic resin, stoneware, and the like. However, in these instances the anode compartment 2 must have a lead plate inserted therein on which the metallic copper anode is placed, the inserted plate ensuring electrical contact.

It is obvious that various types and structures of anodes and cathodes can be employed in the aforescribed cell.

It is thus seen that I have disclosed a method of producing a readily oxidizable copper dust and in embodying this process in making copper sulphate one proceeds as follows:

Employing a cathodic current density of about 600 to about 800 amps. per sq. m., an acidity of about 80 to about 120 grams of sulphuric acid per liter and a cupric ion concentration of about 15 to about 20 grams per liter, the electromotive force of the cell is of the order of 2 to 2.5 volts. The consumption of energy is of the order of 2 to 2.5 kw.-hr. per 1 kg. of dry metallic dust produced.

The metallic dust is by heating it up to about 500° C. to about 600° C. utilizing, for example, an electric oven provided with a temperature regulator and one that is well aired. The consumption of energy for this purpose is 0.2 kw.-hr. per 1 kg. of oxidized dust.

The reaction of the oxide so obtained with sulphuric acid is strongly exothermic. During the reaction in addition to the water and acid required, about one third by volume of the cold saturated solution from the crystallizers should be added. Under these conditions, the acidity is very high and the temperature rapidly rises to 100° C. or more, so that the reaction is rapid and complete. The resulting solution is added to the balance of the cold saturated solution in the crystallizers. This permits a smaller solution circulation.

The method proposed has the following advantages:

(a) The total consumption of energy is comparatively small, being about 0.6 to about 0.8 kw.-hr. per 1 kg. of crystalline copper sulphate produced. Consumption of coal or other fuel is avoided by this method.

(b) The electrolytic cells have no moving parts and are not subject to wear; maintenance presents no problem and the operating personnel required is reduced to a minimum.

(c) During the dissolution of the oxide in the acid it is possible to obtain a very high concen-

tration, thus reducing to a minimum the circulation of the solutions.

(d) The copper sulphate produced is very pure even when produced from scrap copper which contains other metals as impurities. It is very easy to recover precious metals remaining in the anodic sludge.

The form of electrolytic cells described may, in addition to being used for making copper sulphate, be used for the electrolytic production of metallic copper dust, and other metallic dusts.

I claim:

1. The process of preparing a copper dust suitable for conversion to copper sulphate which comprises electrolyzing an electrolyte consisting of free sulphuric acid and cupric ions with a metallic copper anode, the copper being deposited as a fine dust on a cathode, interposing a perforated lead plate anode between the copper anode and the cathode to maintain the concentration of cupric ions in the electrolyte substantially constant throughout the electrolysis, whereby the rate of anodic dissolution of the copper is regulated to be substantially equal to the rate of cathodic deposition of the copper dust, and collecting the precipitated copper dust.

2. The process as claimed in claim 1 wherein the cathodic current density is about 600 to about 800 amperes per square meter, the voltage is 2 to 2.5 volts, and the electrolyte contains about 80 to about 120 grams of sulfuric acid per liter and a cupric ion concentration of about 15 grams per liter.

3. A cell for the preparation of a fine copper dust by electrolysis, said cell comprising an anode compartment containing a metallic copper anode, a cathode compartment containing a cathode on which the copper dust is deposited, a well beneath the cathode for the collection of the copper dust, and a perforated lead plate anode positioned between the anode compartment and the cathode compartment.

NERI CORSINI.

#### REFERENCES CITED

The following references are of record in the file of this patent:

#### UNITED STATES PATENTS

| Number    | Name               | Date           |
|-----------|--------------------|----------------|
| 410,976   | Kerner et al.      | Sept. 10, 1889 |
| 881,580   | Hess               | Mar. 10, 1908  |
| 890,887   | Amenabar           | June 16, 1908  |
| 1,152,772 | Wheeler            | Sept. 7, 1915  |
| 1,777,371 | Koehler            | Oct. 7, 1930   |
| 1,804,924 | Fitzpatrick et al. | May 12, 1931   |
| 1,920,819 | Rose               | Aug. 1, 1933   |
| 2,228,264 | Freedley           | Jan. 14, 1941  |
| 2,326,101 | Nichols            | Aug. 3, 1943   |
| 2,356,897 | Stack              | Aug. 29, 1944  |

#### FOREIGN PATENTS

| Number  | Country       | Date          |
|---------|---------------|---------------|
| 11,800  | Great Britain | Oct. 3, 1885  |
| 255,736 | Great Britain | July 29, 1926 |
| 354,939 | Great Britain | Aug. 20, 1931 |